

## UNITED STATES PATENT OFFICE

2,102,122

FOUNDRY CORE AND DRY BINDER FOR THE  
PREPARATION THEREOF

Fred H. Lane, Hillsdale, N. Y., assignor to Hercules Powder Company, Wilmington, Del., a corporation of Delaware

No Drawing. Application August 12, 1936,  
Serial No. 95,706

## 5 Claims. (Cl. 22—188)

This invention relates to foundry cores and dry binders for the preparation thereof.

Heretofore, in making foundry cores for use in the production of castings, it has been the practice to mix core sand with one of a variety of dry or liquid binders, e. g. pulverized foundry pitch, pulverized rosin, pulverized cereal, pulverized casein, sulfite pulp waste liquor, molasses, sour beer, linseed, soya bean, or other vegetable oil, oil-rosin mixtures, known as core oils, etc. The mixture of sand and binder is then moistened with sufficient water, so that it can be rammed or blown into core boxes of various shapes and sizes, corresponding to the shapes and sizes of cavities it is desired to produce by means of the cores.

When the core box is removed, the grains of sand must be bound together by the binder, so as to permit handling in an approved manner and transferring to an oven. In the oven the cores are then baked to expel the water, drive off volatile constituents, and make the core capable of withstanding ferrostatic pressure encountered in the casting operation.

In casting, the heat of the molten metal burns out the binder, the gases from which vent through the cores and molds, leaving the core in a friable form or as loosely held sand, readily removable from the cavity in the casting when cooled.

Each of the above mentioned core binders has its disadvantages. Foundry pitch has no "green strength" and is also hard to clean from the cavity. Pulverized rosin reverts to solid rosin on storage, i. e. flows together to form a solid mass. Rosin-kerosene-linseed oil mixtures (core oils) tend to crystallize and precipitate the rosin on storage. Cereal binders produce cores which swell, absorb moisture, and give rise to large volumes of acrid smoke in the casting operation. Liquid core binders migrate to the surface of the core and form a hard, impenetrable skin. Linseed oil binder must dry by oxidation, which slows down production. Casein, skimmed milk, etc., are hydroscopic and putrescible when used in cores.

Many attempts have been made heretofore to overcome the above difficulties, but without success.

I have found that a foundry core prepared from core sand, unextracted soybean meal or flour, i. e., soybean meal or flour from which the oil has not been removed by hot pressing or solvent extraction, and gasoline-insoluble pine wood

resin overcomes the above difficulties encountered in the use of old art core binders.

The gasoline-insoluble, pine wood resin I employ in the preparation of my improved core binder and cores made therefrom is hereby defined as the resin such as may be produced from resinous wood, described and claimed in application, Serial No. 61,745, filed January 31, 1936, by Lucius C. Hall, which resin may be produced by extracting resinous wood with a coal tar hydrocarbon, removing said hydrocarbon by evaporation, leaving a residue comprising a mixture of wood rosin and the new resin, extracting wood rosin from said residue by a petroleum hydrocarbon, leaving the new, gasoline-insoluble, pine wood resin.

It will be noted that the unextracted soybean meal used in my improved core binder, contains appreciable, but variable, quantities of soya bean oil which latter enters into the composition.

I have found that pulverized, gasoline-insoluble pine wood resin, as described above, possesses poor green strength when used as a core binder. However, this poor green strength is overcome by the admixture with the toughening unextracted soybean meal or flour. I have also found that while cores made with linseed oil, soybean oil, or other vegetable oils, require long baking at high temperatures, soybean meal or flour, which contains usually about 17% of oil, when mixed with the gasoline-insoluble pine wood resin above described, causes a reaction during the baking, in which the oil and the resin form a condensate, resulting in the production in a short baking period of a high-strength, superior core.

In preparing my improved foundry core composition I mix intimately, for example by grinding together, unextracted soya bean meal and the gasoline-insoluble pine wood resin, hereinbefore described. For example, equal parts thereof may be ground together, and cores made therewith by mixing such composition with foundry sand in a ratio of, for example, 55 parts by weight of sand to 1 part by weight of the composition, and baking the core for about 1.5 hours at about 425° F. The green strength of such cores is satisfactory before baking, and after baking the core has a tensile strength of 177 pounds per square inch. Furthermore, such baked cores may, as a test, be stored in a moisture-saturated atmosphere overnight, and found, after such storage, to have a tensile strength of about 165 pounds per square inch, i. e., a loss of less than 7%. Storage in a moisture-saturated

atmosphere causes a severe loss in strength of cores produced by methods heretofore employed.

Furthermore, I have found that my improved core compositions are practically non-putrescent, due to the presence therein of my special resin, hereinbefore described, which resin contains certain, complex polyphenols, which act as a preservative.

A further advantage of my improved core compositions is that they are dry, and easy to use, as compared to the fluid or semifluid compositions heretofore used.

It will be appreciated that other proportions of ingredients may be used by me in preparing my improved core composition, depending upon the size, type, or complexity of the core it is desired to produce. Nor do I limit myself to the sand/binder ratio or temperature or time of baking, given above by way of example.

It will also be appreciated that I may add additional soybean oil to my core binder composition, or I may use extracted soybean meal and soybean oil, in place of unextracted soybean meal, thus reproducing, in effect, unextracted soybean meal. I may also employ extracted soybean meal and other vegetable oils, such as linseed oil, in place of unextracted soybean meal, and still obtain the advantages, due to the presence of the gasoline-insoluble pine wood resin, of superior strength of core and hardening by condensation effects.

What I claim and desire to protect by Letters Patent is:

1. As a core binder, a mixture of soybean meal containing a vegetable oil, and a gasoline-insoluble, pine wood resin produced by extracting

resinous wood with a coal tar hydrocarbon, removing said hydrocarbon by evaporation, extracting the residue with a petroleum hydrocarbon, and recovering a gasoline-insoluble resin.

2. As a core binder, a mixture of soybean meal, a vegetable oil, and a gasoline-insoluble, pine wood resin produced by extracting resinous wood with a coal tar hydrocarbon, removing said hydrocarbon by evaporation, extracting the residue with a petroleum hydrocarbon, and recovering a gasoline-insoluble resin.

3. As a core binder, a mixture of unextracted soybean meal and a gasoline-insoluble, pine wood resin produced by extracting resinous wood with a coal tar hydrocarbon, removing said hydrocarbon by evaporation, extracting the residue with a petroleum hydrocarbon, and recovering a gasoline-insoluble resin.

4. As a core binder, a mixture of equal parts of unextracted soybean meal and a gasoline-insoluble, pine wood resin intimately mixed together, said pine wood resin being produced by extracting resinous wood with a coal tar hydrocarbon, removing said hydrocarbon by evaporation, extracting the residue with a petroleum hydrocarbon, and recovering a gasoline-insoluble resin.

5. A green foundry core consisting of core sand, unextracted soybean meal and a gasoline-insoluble, pine wood resin produced by extracting resinous wood with a coal tar hydrocarbon, removing said hydrocarbon by evaporation, extracting the residue with a petroleum hydrocarbon, and recovering a gasoline-insoluble resin.

FRED H. LANE.